

## UNITED STATES PATENT OFFICE

2,068,244

## PROCESS FOR THE PRODUCTION OF CASTINGS BY THE CENTRIFUGAL METHOD

Carl Pardun, Gelsenkirchen, Germany, assignor,  
by mesne assignments, to Centrifugal Pipe  
Corporation, Jersey City, N. J., a corporation  
of Delaware

No Drawing. Application February 7, 1935,  
Serial No. 5,403. In Germany March 26, 1934

## 5 Claims. (Cl. 22—192)

This invention relates to a process for the production of castings by the centrifugal method.

In the case of pipes and other castings produced in stationary molds, it has already been proposed to provide the products with a special protective skin by lining the walls of the mold with corrosion-proof materials which penetrate into the surface of the hot mass of the poured material forming the casting, the anti-corrosion properties of said skin being intended to exceed those inherent in the ordinary castings. Acid-resisting metallic alloys have also been proposed for such linings. However, no definite statements have been made respecting the nature of these substances and the manner of their application.

Moreover, in connection with the production of centrifugal castings in chill molds, it has already been proposed to line the rotary molds with ferro-silicon, or ferro-aluminum, prior to the pouring operation. Such lining is intended to modify the quenching action of the walls of the mold and, on the other hand, by reason of its content of silicon or aluminum, to favor the formation of graphite on the outer layer of the pipe, in order to obtain cast pipes with a soft outer skin.

According to the present invention, centrifugally cast pipes with corrosion-proof outer skin can be produced in a centrifugal chill mold by introducing into the mold, prior to casting, a lining composition composed of an alloy of phosphorus which burns or fuses into the external layer of the pipe during the casting process. Alloys of phosphorus with the basic material of the casting can be employed with particular advantage, for example, compositions containing ferro-phosphorus may be used as a lining on centrifugal molds for the casting of iron pipes, or a material containing copper phosphide may be used in the production of copper pipes. The phosphorus alloys are preferably employed in a highly concentrated form, and therefore with a high phosphorus content, it being important to obtain the greatest possible effect from a given quantity of the coating composition.

The distribution of the coating material over the interior wall of the mold is preferably effected by centrifugal force. In order to obtain uniform distribution of the material over the entire length of the rotary mold, it is advisable to employ the coating material in the form of powder and feed it into the mold by means of an axially displaceable charging device. It is also feasible to blow the powdered material into the mold. In some cases it has been found advisable to employ

a binding medium in conjunction with the coating material, to facilitate the adhesion of the powdered material to the wall of the mold. Generally speaking, the amount of the coating composition will be calculated so as to suffice for one casting, and renew it after each casting has been made.

Under the action of the phosphorus, the outer skin of the pipe acquires an increased content of phosphorus, thereby imparting to the said skin a high passivity and powers of resistance to the action of the acids and the like corrosive agents, in the soil. At the same time, ferro-phosphorus has the advantage over other dusting materials that it is easily ground to powder and—in contrast to other ferro-alloys, such as ferro-silicon, ferro-chromium, and the like, which are substantially composed of heavy metals—has a low melting point, inasmuch as one of its components consists of the readily fusible phosphorus. Consequently, other substances applied, in conjunction with ferro-phosphorus, in the form of powder to the surface of the mold, fuse readily into the surface of the basic metal of the casting, since, in this case, the readily fusible phosphorus alloys serve as a flux for other sintering materials of higher melting point.

Copper phosphide, which can also be employed with advantage in the production of centrifugal castings of non-ferrous metallic alloys, has been found to exert a like favorable effect.

Favorable results are for instance obtained with a lining of ferro-phosphorus containing about 20-30% phosphorus and about 80-70% iron. The desired action of the applied ferro-phosphorus begins at a certain minimum amount which depends upon the casting material, and the cross-section and wall-thickness of the articles to be cast. Said lowest amount necessary for producing the desired effect may be easily determined in each particular case. It must, however, be noted that the produced action will be diminished if the ferro-phosphorus is used in amounts which are too large as to be completely absorbed by the casting material. The most favorable effect is produced by using the ferro-phosphorus in the highest amounts which still can be completely dissolved at the temperature and wall-thickness prevailing in each special case. Said maximum moreover depends upon its special composition and more particularly upon the melting-point thereof and its affinity to the casting material. For instance, the favorable amount for a ferro-phosphorus powder of the above mentioned composition (20-30% phosphorus and 80-

70% iron) amounts to between about 30-60 grms. per square meter of the surface of the mold to be lined, in the case of the manufacture of cast iron tubes of an average cross-section and of 5 average wall-thickness.

What I claim and desire to secure by Letters Patent of the United States is:—

1. A process of producing a casting in a centrifugal mold which comprises applying a lining 10 including an alloy of phosphorus to at least a portion of the mold, and then pouring molten metal into the lined mold, thereby forming a casting having the surface which contacted the lining enriched in phosphorus.
- 15 2. A method of producing a casting in a centrifugal mold which comprises applying a lining to at least a portion of the mold surface including a phosphorus alloy of the metal to be cast, and then pouring metal into the rotating mold and 20 over the lining, thereby forming a casting having an exterior surface enriched in phosphorus.

3. A method of producing cast iron pipe in a centrifugal mold which comprises applying a lining of pulverulent material including ferro-phosphorus containing 20 to 30% of phosphorus and 80 to 70% of iron to at least a portion of the mold, and then pouring molten iron over the lining to form a pipe having the surface in contact with the lining enriched in phosphorus.

4. In a method of casting iron in a chilled centrifugal mold, the step which comprises applying to the mold surface pulverulent ferro-phosphorus containing 20 to 30% of phosphorus and 80 to 70% of iron, said pulverulent ferro-phosphorus being applied in an appreciable quantity but not exceeding 60 grams distributed over one 15 square meter of mold surface.

5. A centrifugal mold having at least a portion of the casting surface thereof lined with a pulverulent alloy containing an appreciable percentage of phosphorus.

CARL PARDUN.

20